

May 23, 1933.

P. L. HULIN

1,910,017

ELECTROLYTIC EXTRACTION OF LIGHT METALS CONTAINED IN ALLOYS

Filed Dec. 14, 1928

2 Sheets-Sheet 1



P. L. Hulin  
INVENTOR

By: Marks & Clark  
Attest.

May 23, 1933.

P. L. HULIN

1,910,017

ELECTROLYTIC EXTRACTION OF LIGHT METALS CONTAINED IN ALLOYS

Filed Dec. 14, 1928

2 Sheets-Sheet 2

Fig.2.



P. L. Hulin  
INVENTOR

By: Marks & Clark  
Atts.

## UNITED STATES PATENT OFFICE

PAUL LÉON HULIN, OF GRENOBLE, FRANCE, ASSIGNOR TO COMPAGNIE DE PRODUITS CHIMIQUES ET ELECTROMETALLURGIQUES ALAIS, FROGES ET CAMARGUE, OF PARIS, FRANCE

## ELECTROLYTIC EXTRACTION OF LIGHT METALS CONTAINED IN ALLOYS

Application filed December 14, 1928, Serial No. 325,974, and in France December 21, 1927.

For extracting by electrolysis, from molten substances, a light metal contained in a denser alloy acting as anode, a classical device is known, in which are superposed, in a vat, 5 three molten layers:

The anode, constituted by the dense melted alloy, lying at the bottom and covered by the electrolyte;

The bath or molten electrolyte, of intermediate density, lying between the anode and the cathode;

The cathode, made of light metal released by the electrolyte, floating as a liquid layer or sheet on the bath which it entirely 15 covers.

In this device, the cathode and the anode being in a liquid condition, come in contact, each at its own level, with the side wall of the vat. A short circuit thus exists between 20 both electrodes, through the medium of this wall, and this accident is not uncommon. It is therefore necessary to constitute the said wall in such a manner as to prevent the direct passage of the current through the wall.

25 Now, the latter must also be such that it cannot be disintegrated by the electrolyte.

These conditions present inconsistencies and difficulties of realization which are well known and for overcoming the same various 30 solutions have been proposed.

The present invention has for object to remove the difficulties met with in carrying out the above mentioned classical device.

It is based on the utilization of the principle 35 known in a quite different application according to which the cathode is progressively lifted above the bath and draws along with it the metal which agglomerates thereon in proportion as it is formed, by constituting a 40 solidified rod adhering to the cathode.

The invention is therefore essentially characterized by the combination with a molten anode, which freely extends to the bottom of the electrolysis vat, of a cathode arranged 45 opposite and above the same, and which is prevented from extending to the vat and held out of contact and at a suitable distance from the wall owing to the continuous lifting of the cathode which causes the solidification of the 50 light metal and its concentration in an ag-

glomerated condition in the form of a rod progressively lengthening.

By means of this arrangement any short circuit is avoided as well as any adherence, by contact between the cathode and the wall, 55 and other difficulties.

The side inner wall of the vat can then be lined with a coating of agglomerated carbon, which is the only material known as being capable of suitably resisting in certain baths 60 of melted salts, mainly in those containing alkaline or alkali-earth fluorides.

The invention applies as well to the refining of light metals as to their extraction when they have been produced in the state of alloys. 65

The invention is carried out by means of a suitable plant the arrangements and essential elements of which are diagrammatically illustrated, by way of example only, in the accompanying drawings, Figure 1 and Figure 2.

The system comprises: a metal vat A, made of iron or steel, having a shape variable at will, but preferably a circular shape; the interior of this vat is provided with a lining B, 75 which may be made either of refractory material, or of agglomerated carbon, according to the nature of the electrolytic baths. It is advisable to insert an insulating material between the entire carbon lining and the metal vat. The hearth C, which may be plane or of bowl shape, is made of carbon; it is isolated from the vat and is anodically connected to the electrolytic circuit by a conductor c. The anode-alloy covers the bottom where it forms 80 a molten layer D.

The molten electrolyte is situated immediately above at E.

The cathode is first formed of a metal cylinder F, usually of copper or bronze or 90 similar alloy of good conductivity. It is hung from a metal rod of the same nature f f, freely passing in guides G G and carried by a suspension having a vertical movement of great amplitude, such for instance as a 95 screw a and its toothed nut b, actuated by a worm e.

By means of this suspension, the cathode can be raised, at a reduced and exactly adjusted speed, and have a vertical movement of 100

rather great amplitude. Reversely, it can be lowered at will according to requirements and, in any case, after each operation.

The cathodic current is transmitted there-  
5 to through the rod *f*, either by passing through the guides *G G*, forming or having a sliding contact, or through a flexible conductor, or in any suitable manner.

The anode-alloy *D* is composed of the light  
10 metal to be extracted, incorporated with a heavy metal, much less electro-positive, such for instance as magnesium-lead for extracting magnesium therefrom, or aluminium-copper for extracting aluminium therefrom,  
15 or glucinum-copper for extracting glucinum therefrom, or other similar alloy, for extracting other light metals therefrom.

The electrolyte comprises, either alone, or in admixture in the necessary proportion with  
20 other suitable substances, one or more halogenated compounds, chloride or fluoride, of the light metal to be extracted, the suitable composition, in each case, being either known or easy to determine and does not form a part  
25 of the invention. It is to be noted that the density of the bath must be sufficiently high for preventing the light metal, which has been deposited under the cathode, from becoming detached and from going down again  
30 and that the melting point of the said metal must not be high enough to form and include, in the cathodic deposit, solidified portions of the bath preventing the operation, but this melting point must be, as far as possible,  
35 equal or preferably inferior to the melting point of the light metal which begins to form.

The operation of the new system is as follows:

The bath and the alloy-anode, to be treated,  
40 being brought to molten condition by the usual means, the cylinder *F* is lowered in order to be in contact with the bath without being immersed therein. The electrolysis current is fed to the apparatus and a layer of  
45 fluid light metal *h h* is formed before long under the cathodic cylinder, which metal sometimes overflows about the cylinder, adheres thereto and begins to solidify.

From this moment, by applying to the  
50 new combination: alloy-anode-bath-contacted cathode, the process known under the name of "rising contact cathode", the cathode *F* is slowly raised, according to the well known method, at a speed which is controlled by ob-  
55 serving the two opposed conditions which consist, on the one hand, in not breaking the contact between the bath and the cathode and, on the other hand, in not allowing the latter  
60 to unduly expand or to abandon metal in a separated condition.

On the lower face of the cathode is thus ob-  
tained a deposit of light metal, first fluid and  
65 pasty, which solidifies and, by re-forming it-  
self in the same way and replacing at *h h* the

cylinder *F* in proportion as the latter rises by drawing along the successive layers, finally gives a stick of light coherent metal, of increasing height, as illustrated at *A* in Fig. 2.

This stick is detached and the operation is repeated by bringing back the cathode *F* in contact with the bath.

According to the light metal to be extract-  
70 ed, the lower end of the copper cylinder *F* can be lined with another metal, iron, nickel, al-  
loy, etc., which does not risk of melting or of soiling the metal produced.

When the alloy-anode is sufficiently ex-  
hausted of light metal, the residual part is  
80 evacuated and a new batch of alloy to be  
treated is re-introduced in the vat, or a new  
batch of light metal is re-incorporated on the  
spot with said residual part, if a refining op-  
eration is to be effected.

From the foregoing, it will be seen that the  
object and function of the rising cathode ap-  
plied as stated, notably differ from what they  
are in the old known process.

In fact, in this old process, the object  
sought for is to obtain a very high density of  
current for succeeding in releasing, in a com-  
pact condition, a metal from a salt the elec-  
trolysis of which is effected with difficulty.

In the present invention, the rising cathode  
95 is solely used for localizing the surface of  
the cathodic deposite in order to hold it at  
a sufficient distance from the wall of the vat,  
that is to say for limiting the horizontal ex-  
100 tension of the deposit of the light metal and  
thus preventing the metal, which collects on  
the cathode, from coming in contact with  
the wall of the vat.

In the present application of the rising  
105 cathode to the extraction of the metals which,  
as magnesium and aluminium, admit some-  
what variable current densities, of the aver-  
age order of 1 ampere per square centimeter,  
it is possible to give to this cathode a larger  
110 diameter than in the previous system for the  
case of calcium.

As auxiliary to this increase of diameter,  
a cooling of *F* and, if need be of *H*, can be  
115 effected by any suitable means, such for in-  
stance as by causing the cathode to pass in a  
cooled sheath which surrounds it, without  
hindering its movements.

Ventilated gills and the like can be ar-  
ranged on the cylinder *F*.

A modication which it has not been possi-  
ble to carry out with the side and non metal-  
lic anode of the previous process, consists in  
arranging, on a vat, a number of rising cath-  
odes operating in parallel on the same bath  
125 and opposite one and the same anode. A vat  
thus provided with a group of cathodes will  
have a cross section corresponding to the  
mode of grouping; it could be rectangular  
or oval for instance, and it could thus have  
130

dimensions and a capacity of production notably increased.

The invention further comprises means for obtaining, with the rising cathode, metal sticks having a shape much more regular than was usually heretofore possible.

This means consists in causing the cathode to rotate about its axis at the same time that it rises, that is to say, in imparting to this cathode a movement of rotation on itself in addition to its rising movement.

By the combination of these two simultaneous movements imparted to the cathode, more perfectly cylindrical deposits are obtained in all cases, without prejudicious protuberances as well as a more stable general operation which is better in every respect.

The speed of rotation is not rigorous and can notably vary. There is no need to increase the speed much beyond that which is shown to be sufficient by a trial, in each case, this speed usually corresponding to a few revolutions per minute.

The mechanism necessary for this rotary movement added to the vertical movement with the accessories embodied in the whole structure (friction contacts, driving members, etc.) are easy to devise and need not be described, as they can assume varied shapes and arrangements which do not form a part of the invention.

All the details for carrying out the invention may be varied according to circumstances without altering the principle of the said invention.

I claim:

1. An apparatus for the electrolytic extraction by means of fusion of light metals comprising a vat, an anode of molten metal of an alloy of the metal to be extracted, an electrolyte and a rising cathode formed by the solidified extracted metal.

2. An apparatus for the electrolytic extraction by means of fusion of light metals comprising a vat, an anode of molten metal of an alloy of the metal to be extracted, an electrolyte and a rising cathode formed by the solidified extracted metal, the cathode being formed by multiple rods disposed in parallel opposite the single anode in a molten alloy.

3. An apparatus for the electrolytic extraction by means of fusion of light metals comprising a vat, an anode of molten metal of an alloy of the metal to be extracted, an electrolyte and a rising cathode formed by the solidified extracted metal, and means for imparting a movement of rotation to the rising cathode.

4. An apparatus for the electrolytic extraction by means of fusion of light metals comprising a vat, an anode of molten metal of an alloy of the metal to be extracted, an electrolyte and a rising cathode formed by the solidified extracted metal and a frame or lining of carbon on a level with the upper layer.

The foregoing specification of my "Improvement in the electrolytic extraction of light metals contained in alloys"; signed by me this thirtieth day of November 1928.

PAUL LÉON HULIN. 70

75

80

85

90

95

100

105

110

115

120

125

130